

# UNITED STATES PATENT OFFICE.

JOHN FOTTRELL, OF PHILADELPHIA, PENNSYLVANIA.

## INSULATING MATERIAL.

SPECIFICATION forming part of Letters Patent No. 433,893, dated August 5, 1890.

Application filed December 23, 1889. Serial No. 334,738. (No specimens.)

*To all whom it may concern:*

Be it known that I, JOHN FOTTRELL, a citizen of the United States, residing at Philadelphia, in the county of Philadelphia and State of Pennsylvania, have invented certain new and useful Improvements in Insulating Material; and I do declare the following to be a full, clear, and exact description of the invention, such as will enable others skilled in the art to which it appertains to make and use the same.

My invention relates to the insulation of electrical conductors; and its object is to obtain an insulating material which is substantially equal to rubber, but which is cheaper, firmer, and more durable than rubber, and which does not require vulcanization. I attain this object by thoroughly mixing together in any suitable manner india-rubber and aluminum oleate. Aluminum oleate is best prepared by precipitating a solution of sodium oleate or soap with a solution of aluminum sulphate or alum, expressing the water from the spongy precipitate, and then drying it at a moderate temperature. Palm-oil soap is best for this purpose, and in general the perfection of the resulting composition depends on the purity of the ingredients, though I have found that any form of

rubber may be used, provided that it is thoroughly mixed with the aluminum oleate. When so mixed, the compound is homogeneous, and experiment indicates that under the action of the electric current it improves in quality and its insulating resistance is increased.

For ordinary use the rubber and aluminum oleate are mixed together in equal parts, by weight; but these proportions may be varied, a larger proportion of the rubber giving greater flexibility to the compound. Ordinarily no vulcanization is necessary, though the compound is susceptible of vulcanization, if desired.

Having thus fully described my invention, what I claim, and desire to secure by Letters Patent, is—

An insulating material for electrical conductors, consisting of a mixture of india-rubber and aluminum oleate, substantially as described.

In testimony whereof I affix my signature in presence of two witnesses.

JOHN FOTTRELL.

Witnesses:

D. A. MCKNIGHT,  
WILLIAM H. BOOZ.